

# UNITED STATES PATENT OFFICE.

CHARLES GERHARD, OF JERSEY CITY, NEW JERSEY.

## BENGAL-LIGHT COMPOUND.

SPECIFICATION forming part of Letters Patent No. 449,530, dated March 31, 1891.

Application filed January 22, 1891. Serial No. 378,700. (No specimens.)

*To all whom it may concern:*

Be it known that I, CHARLES GERHARD, a citizen of the United States, residing at Jersey City, in the county of Hudson and State 5 of New Jersey, have invented new and useful Improvements in Compounds for Bengal Lights, of which the following is a specification.

This invention relates to a compound produced by copal, ether, alcohol, nitrate of strontia, chlorate of potash, and shellac solution.

In carrying out my invention I take ten pounds of copal and add thereto sufficient ether to cover the copal. By comminuting the 15 copal the process is expedited. I have found a convenient way to be to spread the copal over the bottom of a vessel, to then add the ether, and occasionally stir the mass. When the mixture of copal and ether becomes of a 20 jelly-like consistence, I add a gallon of alcohol and heat the mixture to the boiling-point. To the mixture thus produced I add forty pounds nitrate of strontia and ten pounds of chlorate of potash, and also about a gallon 25 and a half of alcoholic solution of shellac or varnish. When this mixture has become set or hardened, it is ready for use. I have found that the shellac can be dispensed with and the compound will then burn with equal brilliancy; but an advantage of adding the shellac is that by such addition the generation of 30 smoke or vapor is diminished or obviated.

The ether is a well-known solvent of copal or resin; but in place of ether any of its well-known equivalents can be used, such as linseed-oil, hemp-oil, nut-oil, poppy-oil, turpentine-oil, oil of rosemary, benzole, photogen, or acetone.

The manner of using the compound is simi-

lar to that of using any Bengal-light compound, such as putting the compound in a box or shell and lighting it when required or applying the compound to the end of a handle or torch for convenient use. By providing the end of the handle or torch with a paper tube or shell and placing the compound in the shell with a suitably-projecting fuse or slow match the compound will always be in position to be lighted.

The advantages of the mixture are that the copal is a resinous substance which offers great resistance to influences of the weather, and being treated with ether and alcohol it forms a weather-proof varnish, and torches or pyrotechnical preparations coated with this varnish will keep in any climate or weather.

The compound prepared according to the above specification can be exposed to atmospheric changes without deteriorating.

What I claim as new, and desire to secure by Letters Patent, is—

1. A compound for Bengal lights, consisting of copal, ether, alcohol, nitrate of strontia, and chlorate of potash, substantially in the proportion above described.

2. A compound for Bengal lights, consisting of copal, ether, alcohol, nitrate of strontia, chlorate of potash, and shellac solution or varnish, substantially in the proportion above described.

In testimony whereof I have hereunto set my hand in the presence of two subscribing witnesses.

CHARLES GERHARD.

Witnesses:

WM. C. HAUFF,  
E. F. KASTENHUBER.